

June 19, 1923.

1,459,357

M. C. BOOZE

CERAMIC ARTICLE AND METHOD OF MAKING THE SAME

Original Filed Feb. 17, 1921



Witnesses

John H. Glenna  
Leah A. Sessions

Inventor

Macdonald C. Booze

By Clayton H. Booze  
Attorney.

## UNITED STATES PATENT OFFICE.

MACDONALD C. BOOZE, OF WORCESTER, MASSACHUSETTS, ASSIGNOR TO NORTON COMPANY, OF WORCESTER, MASSACHUSETTS, A CORPORATION OF MASSACHUSETTS.

## CERAMIC ARTICLE AND METHOD OF MAKING THE SAME.

Application filed February 17, 1921, Serial No. 445,833. Renewed December 8, 1921. Serial No. 520,991.

To all whom it may concern:

Be it known that I, MACDONALD C. BOOZE, a citizen of the United States of America, residing at Worcester, in the county of Worcester and State of Massachusetts, have invented certain new and useful Improvements in Ceramic Articles and Methods of Making the Same, of which the following is a full, clear, and exact specification.

- 10 My invention relates to a laminated article comprising ceramic bonded granular material and to a process of making the same, and more particularly to a multilayer article which has an exposed or working face 15 portion of a special composition and character to meet specific chemical, refractory or abrasive requirements, while the backing and bulk of the article is made of a cheaper and more easily fabricated material.
- 20 Certain uses of refractories, abrasive stones or non-slip tiles make it desirable or necessary that the face portion only of the article contain super-refractory or abrasive material. For example, a brick intended to 25 be exposed to the destructive action of chemical gases, slag or molten baths, may have one face consisting mainly of crystalline alumina and the other face substantially the same as a fire brick. It also is not eco- 30 nomically expedient to provide such an article with the expensive super-refractory or abrasive material throughout the entire structure where it is necessary that the surface portion only be of this protective or 35 abrasive nature.

It has been proposed to make a refractory article of several layers containing silicon carbide in such decreasing amounts from the facing towards the rear as will give a graduated and increasing coefficient of expansion. It is found, however, that such procedure results in a warped article if it is fired at such a high temperature as to cause 40 material shrinkage of the clay backing, it being evident that the silicon carbide facing will not shrink to the same extent as does the clay.

It is accordingly an object of my invention to overcome the objectionable features found 45 in prior articles of this type and to produce a multilayer article which has a refractory

or abrasive surface portion integrally united with a backing of a less refractory or abrasive mixture which may be fired at high temperatures without detrimental warpage 55 and will be more economical than and as serviceable as an article which has a uniform structure throughout.

A further object of my invention is to provide a feasible and economical method of 60 forming a ceramic article of the class described by substantially equalizing the drying and burning shrinkages in the different portions of such a multilayer body whereby a facing containing a high content of pre- 65 shrunk grains may remain integrally united with a backing of a different composition and the latter will not crack away or shrink to such an extent as to render the article defective. Other objects will be ap- 70 parent in the following disclosure.

In accordance with my invention, I propose to make articles of this class by employing such compositions and methods of operation as will increase the drying and burning 75 shrinkage of a ceramic body containing super-refractory material of low shrinkage value and to provide a multiple layer article by supplementing such procedure with that involved in decreasing the shrinkage of the 80 portion which would normally shrink too much for use in an article of this type, or I may employ only the latter method of equalizing shrinkage. I furthermore preferably employ one or more intermediate 85 layers of suitable compositions to avoid abrupt shrinkage differentials during drying and firing. The shrinkage of the facing is increased by employing a large amount of water with the bond, while the 90 backing may be maintained in a comparatively dry state so that elimination of moisture will not materially affect the size of this portion of the article.

The most efficient preshrunk super-refractory materials adapted for refractory or abrasive purposes comprise such substances as silicon carbide, crystalline alumina, etc., and this invention is broadly applicable to all super-refractory and abrasive materials 100 which may be bonded by ceramic bonds of the class herein described although my

method is described herein with particular reference to but one of them. Crystalline alumina, which occurs in nature as corundum or in the various emerys and may be 5 made artificially by fusing and crystallizing such substances as bauxite, containing various types and degrees of impurities adapted to modify the temper, the physical characteristics and the chemical composition of 10 the crystallized grains, does not shrink materially when fired in the ordinary ceramic kiln, whereas the various clay materials used as bonds for the refractory grains and employed by themselves to form fire bricks 15 have a large shrinkage during drying and burning. Hence, if one wishes to provide a fire brick or abrasive block with a facing of crystalline alumina, it is necessary to compensate for the difference of shrinkages during 20 the manufacturing operations.

As one method of increasing the shrinkage of the facing of the article, which consists essentially of super-refractory grains such as crystalline alumina, I propose to utilize 25 a ceramic bond therefor which contains an ingredient capable of providing a large degree of shrinkage during drying and preferably during both the drying and the burning operations. A substance admirably 30 adapted for my purposes is bentonite, which is a peculiar variety of clay found in the State of Wyoming, and is characterized mainly by the property of absorbing about three times its weight of water and swelling 35 to a marked extent. While this clay varies considerably in composition, it ordinarily is of a yellowish green color when fresh and assumes a light green to white color on exposure to the atmosphere. The clay, which 40 has a specific gravity of about 2.18, is exceedingly fine grained and soft and is thought by some to be in a colloidal condition. A typical analysis of one of these clays is as follows:

|    |                                      |        |
|----|--------------------------------------|--------|
| 45 | Al <sub>2</sub> O <sub>3</sub> ----- | 18.97% |
|    | Fe <sub>2</sub> O <sub>3</sub> ----- | 1.85   |
|    | SiO <sub>2</sub> -----               | 64.58  |
|    | TiO <sub>2</sub> -----               | 0.20   |
| 50 | CaO -----                            | 0.63   |
|    | MgO -----                            | 2.03   |
|    | SO <sub>3</sub> -----                | 0.69   |
|    | H <sub>2</sub> O -----               | 8.08   |
| 55 | Na <sub>2</sub> O } -----            | 1.06   |
|    | K <sub>2</sub> O } -----             |        |

By incorporating bentonite in the plastic clay material with which the alumina grains are bonded, I insure that upon mixing with water the alumina grains will be separated 60 by the swelling of the bond, so that upon drying and burning, the mass will shrink more than if bentonite were not present. The rear portion of the article not containing this bentonite will shrink the normal 65 amount, according to its composition.

Hence, by a proper adjustment of the amounts of bentonite used and the water contents of the different layers, I may so adjust the shrinkage values of the different portions that they will be substantially 70 equalized.

I furthermore compensate for this shrinkage differential by incorporating in the backing a preshrunk refractory material in such proportions as to reduce the shrinkage of this 75 layer to the desired extent. An inexpensive material suitable for my purpose is fire clay grog, obtained by breaking up old saggers and batts which have previously been fired at a temperature as high as that to which 80 the new article will be heated, whereby the grog has been shrunk substantially to its maximum extent, before use in the new article. The proportions of the refractory grog are determined by various factors, such 85 as the nature of the clay materials employed and the amount of shrinkage compensation desired. I, however, find that for this type of refractory I ordinarily utilize an amount of granulated grog far in excess of that 90 heretofore specified and deemed the maximum for firebrick compositions. This is made possible by the use of a ball clay considerably more plastic than the clays commonly employed in making fire bricks. It 95 will be evident that if intermediate layers are employed, these will be made up of mixtures of the ingredients of the surface layers, with the essential materials affecting the shrinkage decreasing in amount from 100 one face toward the other, so that all the layers will shrink to substantially the same extent.

As a specific embodiment of my invention, reference is to be had to the accompanying 105 drawing which shows in a cross sectional view a refractory brick made up of three layers, a front facing 1 consisting essentially of crystalline alumina bonded by a vitreous ceramic material, a refractory clay 110 backing 2 such as burned fire clay and grog and an intermediate layer 3 of a mixture of the ingredients of the two outer portions. As a specific example of a composition which 115 will be suitable for a fire brick capable of withstanding heat treatment at Seger cone 15, as determined largely by the refractoriness of the backing, the following table of ingredients and proportions is to be noted:

#### 120 Facing.

##### Crystalline alumina grains

|                         |               |
|-------------------------|---------------|
| 14 mesh and finer ----- | 84% by weight |
| Ball clay -----         | 15% by weight |
| Bentonite -----         | 1% by weight  |

#### 125 Intermediate layer.

|                           |               |
|---------------------------|---------------|
| Crystalline alumina ----- | 35% by weight |
| Fire clay grog -----      | 45% by weight |
| Ball clay -----           | 20% by weight |

*Backing.*

Fire clay grog 10 mesh and  
finer ----- 75% by weight.  
5 Ball clay ----- 25% by weight.

Water for each batch to give desired plasticity.

These ingredients are combined in accordance with well known ceramic methods of 10 mixing, shaping and firing, it being noted that the low plasticity of the mixture ordinarily requires forming the superimposed layers of the article by tamping or pressing. The ingredients of each layer are mixed 15 up separately and after the first layer has been tamped in the mold, it is levelled off and then given a slightly rough surface to insure better uniting with the adjacent layer, the next layer placed on it and similarly 20 treated, and so on. It is to be noted that the facing material is mixed with a large amount of water while the backing is kept as dry as is feasible to further reduce the differential shrinkage. The article is then 25 dried by the ordinary methods and fired at about cone 12 to vitrify the bond in the facing in accordance with the usual procedure.

By carrying out the above procedure, I 30 provide a block in which the facing is made up substantially of crystalline alumina grains bonded by vitrified clay material, the grains having been drawn together by the shrinking of the clay bond during drying and firing so that they are in substantial 35 contact. The vitrified ceramic material, which may be modified as desired to form either a nonglassy or a vitreous bond, is present mainly in the interstices between the 40 grains and unites integrally therewith, as is well understood in this art. The backing made by the specific formula given is similar to a fire clay brick but has a higher content of grog than ordinarily employed. 45 The intermediate layer is made up of a mixture of the ingredients and has somewhat of the physical characteristics of each outer layer.

In an article formed of the above composition, the facing bond is in a non-glassy condition. For certain types of abrasive articles, it is desirable that the bond be of a vitreous nature. In this case, slip clay and other low melting substances may be 55 used in the bond for the abrasive granules, the low melting ingredient serving to lower the fusion point of the mass to the firing temperature of the ceramic kiln. Owing to these ingredients being ordinarily employed in large amounts such as 20% of the mass by weight, and causing a high shrinkage of the facing, the low shrinking material in the backing may be materially reduced in amount.

55 It will be obvious that changes may be

made in the ingredients used and that the proportions of the different materials may be varied widely within the scope of the appended claims without departing from the spirit of this invention. For instance, 70 the amount of bentonite employed will depend upon the characteristics and proportions of the ingredients present in the other layers as well as the degree of shrinkage compensation desired. It will also be evident that I am not equalizing the shrinkage of the different portions of this brick for any temperature which may be employed, but that such equalization refers only to the 75 temperature at which the brick is intended to be fired or used, it of course being obvious that it is not necessary, within the scope of this invention, that the shrinkage of the different layers be exactly alike. If the brick is to be used for abrasive purposes 80 or as a non-slip tile, then the temperature under consideration is that of the firing temperature, and if it is to be employed as a refractory then the shrinkage will be equalized for a temperature of a few cones 85 higher than that of burning. Furthermore, it is clear that the super-refractory materials covered by my claims are those which are capable of withstanding the temperature of firing the multilayer article as determined 90 by the nature of the clay materials present therein and of serving the purposes desired for the finished product.

Having thus described my invention, what I claim as new and desire to secure by Letters Patent is:

1. The method of making a multilayer ceramic article having a facing of bonded granular material, comprising the steps of incorporating with said granular material 105 a ceramic bond containing an ingredient capable of producing high drying shrinkage, adding water thereto to make a plastic mass, adding a backing of ceramic material, shaping the article, drying the same, and subsequently firing the mass to bond the granules together and unite the backing therewith.

2. The method of making a multi-layer ceramic article having a super-refractory facing and a less refractory backing comprising the steps of superimposing a backing of plastic ceramic material and a facing of pre-shrunk refractory granules incorporated with a ceramic bond containing an ingredient capable of high drying shrinkage and of equalizing the shrinkage of the two layers during the firing operation and thereafter drying and firing the mass to bond said granules and unite the backing therewith. 115 120

3. The method of making a multilayer article containing super-refractory grains in one face portion only, comprising the steps of incorporating with said grains a ceramic bond containing a clay of normal shrinkage 130

and an ingredient capable of causing abnormally high shrinkage of the bond during drying and burning, forming a moldable plastic mixture thereof, providing a layer of 5 said bonded mixture with a backing of ceramic material and firing the article to bond the grains together and unite the backing integrally therewith.

4. The method of making a multilayer 10 article, comprising the steps of incorporating with super-refractory granular material a vitrifiable ceramic bond containing an ingredient capable of swelling greatly when wetted with water, forming a plastic mixture 15 thereof in which the grains are separated by the swollen ceramic medium, providing a ceramic backing layer therefor, drying the article, and thereafter firing the article to vitrify the ceramic bond adjacent the granules and unite the backing integrally therewith.

5. The method of making an article of ceramic bonded granular material, comprising the steps of mixing said material with 25 a vitrifiable clay and bentonite, adding water thereto to form a plastic mass, shaping the article, drying the same to cause a partial shrinkage, and thereafter firing the mass to vitrify the bond and unite the granular 30 material into an integral mass.

6. The method of manufacturing an article which has a facing containing super-refractory grains and a backing of a different composition, comprising the steps of incorporating with said grains a vitrifiable 35 ceramic bond having a high drying shrinkage, providing a backing of clay and refractory granules of low shrinkage value proportioned in amount to compensate for the high shrinkage value of said clay and to 40 equalize the shrinkage of the facing and backing, and firing the layers in superimposed relation to bond the super-refractory grains and unite said backing integrally 45 therewith.

7. The method of forming a multilayer article, comprising the steps of incorporating with granular super-refractory material a vitrifiable clay and a material capable of increasing the drying shrinkage of the mass, 50 adding water thereto and forming a layer from the plastic mixture, mixing fire clay with a preshrunk ingredient capable of reducing shrinkage of the mixture during drying and burning, forming a backing thereof adjacent the granular facing, drying the article, and thereafter firing the article to vitrify the ceramic bond and unite the fire clay backing therewith.

8. The method of forming a multilayer 55 article containing a preshrunk super-refractory granular material in its face portion, comprising the steps of incorporating with said granular material a vitrifiable ceramic bond capable of large shrinkage during dry-

ing and burning, providing a backing composition of fire clay and refractory granules of low shrinkage value, proportioning the amounts of the bond and said granules to substantially equalize the shrinkage of the 70 two layers when fired to vitrify the bond, forming plastic superimposed layers therefrom, drying the article, and thereafter firing it at a temperature to vitrify the ceramic bond and unite the backing integrally therewith.

9. The method of forming a multilayer 75 ceramic article, comprising the steps of incorporating with super-refractory granular material a ceramic bond containing bentonite, providing a backing therefor of plastic ceramic material, drying the article, and firing to bond said granules and unite the backing integrally therewith.

10. The method of forming a multilayer 80 article, comprising the steps of mixing crystalline alumina grains with a vitrifiable clay and a material capable of high drying shrinkage, adding water thereto and forming a plastic mixture thereof, shaping a 85 layer therefrom, providing a ceramic backing therefor of lower refractoriness, drying the article, and firing to vitrify the bond and unite the backing thereto.

11. The method of forming a multilayer 90 article, comprising the steps of incorporating with super-refractory granular material a vitrifiable ceramic bond containing an ingredient capable of high drying shrinkage, forming a plastic mixture thereof as one 95 layer of the article, superimposing therewith a backing layer of fire clay and fire clay grog, and drying and firing the article to vitrify the clay bond and unite the layers into an integral mass.

12. The method of forming a multilayer 100 article, comprising the steps of incorporating with super-refractory granular material a vitrifiable ceramic bond containing an ingredient capable of producing high 105 drying shrinkage, forming a plastic mixture thereof as one layer of the article, superimposing thereover a layer containing a smaller amount of said super-refractory material and a larger proportion of ceramic 110 material, forming a backing layer thereover of fire clay and fire clay grog, and drying and firing the article to vitrify the clay bond and unite the layers into an integral 115 mass.

13. The method of forming a multilayer 120 article, comprising the steps of mixing crystalline alumina with a vitrifiable clay and bentonite, adding water and forming a plastic layer thereof, superimposing thereover a 125 backing of vitrifiable clay and pulverized fire clay grog, drying the article, and subsequently firing at a temperature to vitrify the ceramic bond and unite the backing integrally therewith.

14. An article of manufacture having a facing comprising crystalline alumina granules and a vitrified ceramic bond therefor containing an ingredient of high drying shrinkage, and a backing comprising granules of low refractoriness and burned fire clay integrally united with the facing.
15. An article of manufacture having a facing comprising crystalline alumina granules, a vitrified ceramic bond therefor, and a backing comprising burned fire clay and granulated fire clay grog united with the facing by an intermediate layer of burned ceramic material.
16. An article of manufacture having a facing comprising crystalline alumina granules and a vitrified ceramic bond therefor, a backing comprising burned fire clay and grog, and an intermediate layer between the facing and backing comprising burned ceramic material integrally uniting the two outer layers, said layers having had substantially the same shrinkage during drying and burning.
17. An article of manufacture having a facing comprising crystalline alumina granules, a vitrified ceramic bond therefor, a backing integrally united therewith by a burned ceramic material comprising fire clay and a preshrunk granular material of lower refractory value than that of the alumina granules, the ingredients thereof being so selected that the drying and burning shrinkage of the facing substantially equals the shrinkage of the backing.
18. An article of manufacture having a facing comprising crystalline alumina granules, a vitrified ceramic bond therefor, a backing comprising crushed grog and burned fire clay, and an intermediate layer containing fire clay, grog and alumina in lesser amounts than the outer shrinkage of adjacent layers, the layers of the article having been substantially equalized.

Signed at Worcester, Massachusetts, this 15th day of Feb. 1921.

MACDONALD C. BOOZE.

**Certificate of Correction.**

It is hereby certified that in Letters Patent No. 1,459,357, granted June 19, 1923, upon the application of MacDonald C. Booze, of Worcester, Massachusetts, for an improvement in "Ceramic Articles and Methods of Making the Same," an error appears in the printed specification requiring correction as follows: Page 5, strike out present lines 42 and 43, claim 18, and insert instead *lesser amounts than the outer layers, the shrinkage of adjacent layers of the article*; and that the said Letters Patent should be read with this correction therein that the same may conform to the record of the case in the Patent Office.

Signed and sealed this 24th day of July, A. D., 1923.

[~~SMAL.~~]

WM. A. KINNAN,  
*Acting Commissioner of Patents.*